

# UNITED STATES PATENT OFFICE.

FRANK C. WHEELER, OF MONTREAL, QUEBEC, CANADA.

## METHOD AND COMPOSITION FOR RENDERING MATERIALS FIREPROOF.

1,414,609.

Specification of Letters Patent.

Patented May 2, 1922.

No Drawing.

Application filed September 18, 1917. Serial No. 192,003.

*To all whom it may concern:*

Be it known that I, FRANK C. WHEELER, a subject of the King of Great Britain, and resident of the city of Montreal, in the Province of Quebec and Dominion of Canada, have invented certain new and useful Improvements in Methods and Compositions for Rendering Materials Fireproof, of which the following is a full, clear, and exact

10 description.

This invention relates to a composition for rendering materials of various kinds fireproof, and also to the method or process for applying the fireproofing composition to various materials.

15 It has been found very desirable to fireproof such articles as textile fabrics, and recently it has become more and more imperative that many materials should be rendered fireproof to prevent destruction from explosions and other incendiary causes.

The composition which I use may be applied not only to fabrics but to raw materials, as well as articles of wood, paper and

20 fibrous products.

The main constituent or base of the fireproofing material is borax, which may be used either in solution or in its powdered form, but preferably in solution. The borax

25 solves readily in water, and may be used in quantities ranging from one-quarter of a pound to one pound per gallon of water. To this solution may be added from one to two ounces of commercial alum, the strength

30 of the solution depending largely on the texture of the material to be treated. In applying the composition to fabrics and the like, the materials are placed in a suitable

reservoir or tank containing the proper amount of solution, and disposed in such 40 manner as to enable the solution to reach every part of the material. The temperature of the contents of the tank is then raised to boiling point for a period of approximately one hour. For loosely woven fabrics, the boiling process may be shortened 45 slightly, and for very heavy or tightly woven materials, the time of boiling may be increased. Raw materials such as cotton, wool, kapok and the like may be similarly treated, 50 and such fibrous materials as wood, paper, paper board and the like may be treated by immersing the articles in the solution until they become impregnated.

In some cases where the boiling treatment 55 is impracticable or inconvenient, a mixture of powdered borax and alum may be sprinkled or blown over the surface of the materials. This method may be found particularly advantageous in treating bales of 60 cotton, kapoc and the like.

Having thus described my invention, what I claim is:—

1. A fireproofing material comprising the composition resulting from the mixing of 65 borax, alum and water in the proportions of 4 to 16 ounces borax, 1 to 2 ounces alum and 1 gallon water.

2. A method of fireproofing, which comprises immersing the material to be fireproofed in a composition resulting from the mixing of water, borax and alum, and boiling for approximately one hour.

In witness whereof, I have hereunto set my hand.

FRANK C. WHEELER.